

W. A. KNAPP,  
ART OF PERMANENTLY HEAT EXPANDING CAST IRON ARTICLES,  
APPLICATION FILED OCT. 28, 1915.

1,274,896.

Patented Aug. 6, 1918.

Fig. 1.



Fig. 2.



Fig. 3.



Inventor

William A. Knapp

By

John S. Barker

his Attorney

Witnesses

Marshall Low

# UNITED STATES PATENT OFFICE.

WILLIAM A. KNAPP, OF WASHINGTON, DISTRICT OF COLUMBIA, ASSIGNOR, BY DIRECT AND MESNE ASSIGNMENTS, TO CHARLES SCHWARTZ, TRUSTEE, OF WASHINGTON, DISTRICT OF COLUMBIA.

## ART OF PERMANENTLY HEAT-EXPANDING CAST-IRON ARTICLES.

1,274,896.

Specification of Letters Patent.

Patented Aug. 6, 1918.

Original application filed October 7, 1915, Serial No. 54,613. Divided and this application filed October 28, 1915. Serial No. 58,444.

To all whom it may concern:

Be it known that I, WILLIAM A. KNAPP, a citizen of the United States, residing at Washington, District of Columbia, have invented certain new and useful Improvements in the Art of Permanently Heat-Expanding Cast-Iron Articles, of which the following is a specification.

My invention relates to a process of treating finished cast iron articles by which they are permanently heat-expanded, and consists of the process herein to be described and to the products of such process.

I have discovered that iron castings, when subjected to a red heat and then allowed to cool slowly, may become permanently expanded, that is to say, they do not, upon cooling, contract to the same sizes as they had before being heated, but remain permanently enlarged to a perceptible degree. I believe that this is true of all kinds of iron castings, but the tendency to expand permanently is particularly pronounced in hollow castings, and more especially in those of cylindrical form, such as gas engine pistons. Furthermore, I have also discovered that castings so expanded may be again permanently expanded and the process repeated until a substantial degree of enlargement is secured.

I have applied my invention practically to the expansion and refitting of worn or loose cast iron engine pistons, particularly to the pistons of gas engines, and more especially to those of engines used upon motor vehicles; and I shall in this application describe the process in connection with the expanding of and refitting of such pistons, although the principle of the invention may be applied to advantage to the fitting of new pistons and cylinders, and to the expanding and fitting of other articles than pistons.

In the accompanying drawings—

Figure 1 is a longitudinal sectional view through the cylinder of an internal combustion engine, which has been used until the cylinder has become so worn that the piston no longer fits it accurately and tightly, the view being largely diagrammatic in its character, and the showing of the extent to which the cylinder is worn exaggerated;

Fig. 2 is a view illustrating one method of heating a piston to expand it; and

Fig. 3 is an elevation illustrative of the cooling step of the process. 55

In the expanding of an ordinary iron casting, such as the piston of an engine, I heat it to a temperature of between 1400 and 1600 degrees F. This heating may be in a furnace or a retort, or it may be by means of a blow torch. The latter method is illustrated in Fig. 2 where *a* indicates a hollow gas engine piston, *b* a jacket of non-cumbustible, heat-insulating material, such as asbestos, *c* a hot bed, as of glowing charcoal, upon which the incased piston is seated, and *d* a blow torch delivering flame into the interior of the piston for heating it. The illustration in Fig. 2 is typical, though practical and one that has been employed by me. 60 70

When the article being heated has been raised to the desired temperature the application of heat is discontinued and the casting allowed to cool slowly. This may be accomplished by removing the torch and covering the open end of the piston, as by means of a sheet of asbestos, such as indicated at *e* in Fig. 3. The jacket *b* and covering *e* not only insure a gradual and uniform cooling, but largely operate to prevent access of air 75 80 to the article *a*, thus reducing the liability of the surfaces of the piston becoming oxidized and scaling.

On becoming cooled the casting will be found to have expanded slightly in all directions, and this expansion I have discovered remains permanent. If the expansion secured by a single heat treatment as described is insufficient for the purpose in view, the treatment is repeated, with the result that the casting will be again, and further, enlarged, the second expansion being also permanent, and this alternate heating and cooling may be carried on with safety a number of times so as to secure a 85 90 95 considerable enlargement of the article.

One extremely useful and valuable application of my invention is to the refitting of pistons to engine cylinders where one or both have become worn. I refer to Fig. 1 100 of the drawings where *a* indicates the piston of a gas engine, and *f* the cylinder in which it works, these, particularly the cylinder, having become, through use, so worn that the piston no longer fits the cylinder tightly. 105 In practice the piston of a gas engine be-

comes somewhat reduced in diameter through wear, and the cylinder in which it works becomes enlarged, particularly at those parts opposite which the piston travels, as indicated at *g* in Fig. 1, so that the cylinder chamber becomes larger at the rear parts *g* than at the front portion *h*. When this occurs it is now the common practice to obtain a new, "oversize" piston, and to 10 rebore the cylinder to fit such piston. This practice is expensive and not always satisfactory, as the reboring is often attempted upon a machine not especially intended for that purpose, with the result that the engine 15 cylinders are frequently seriously injured. Furthermore, the balance of the engine by the use of an oversize piston is disturbed, and this is believed by some to injuriously affect the running of an engine thus 20 equipped.

By the use of my invention I am enabled to overcome the objections to the use of an oversize piston replacing one that has become worn, to materially reduce the expense 25 incident to the installation of such a piston, and to insure a uniformly better result. To secure this I expand the worn piston, according to the method already herein described, until it fits closely the outer portion 30 *h* of the cylinder. I then insert this expanded piston into the open end of the cylinder, and grind the latter, by means, for instance, of the piston, using some abrasive between them, taking off the high places 35 and irregularities of the cylinder and bringing it to true cylindrical shape and to a slightly greater diameter than it originally had. If a single grinding be not sufficient the piston is a second time expanded and 40 the grinding and shaping process just described repeated, and this is continued until the cylinder throughout its working portion is brought to true cylindrical shape and of the desired diameter to fit the piston. Two 45 or three alternate expanding and grinding operations have been usually found to be sufficient to restore a considerably worn cylinder to good working condition. Should the expansion of the piston at any time be 50 found too great to permit of its insertion into the end *h* of the cylinder, it may be reduced in diameter by turning. Not only is the process useful in refitting old pistons to old cylinders, but it will be found 55 of advantage in obtaining a perfect fit between new cylinders and new pistons.

It is well understood that a better fit is obtained by grinding two parts together than where it is sought to secure the desired 60 result by turning processes alone, and by my process the fitting, by the grinding together of cylinder and piston, is easily made practically possible.

The temperatures to which the articles 65 being treated according to my process are

heated, hereinbefore mentioned, that is, between 1400 and 1600 degrees F. are those that I have found the most practical under ordinary conditions, but they do not mark the limits of the temperatures between which 70 my invention may be worked, because I have found that a temperature as low as about 1200° F. will cause a slight permanent expansion of an article subjected to that heat and treated according to the process herein described, and such relatively low temperature, or one between that and 1400° F. may be to advantage employed where a very slight expansion is desired. While I am not now able to fix the limits of temperature 75 for heating the articles when practicing my process, with accuracy, I believe that the term red heat describes with approximate accuracy the range of temperatures available for the heating step of the 80 process.

I am aware that for some time has been known the fact that cast iron articles when heated to a temperature of about 900 to 1200° F. and then allowed to cool become 85 permanently expanded, this fact having been noticed in connection with a method of operating upon chilled iron castings, such as car wheels, for the purpose of increasing the strength of the metal and relieving the 90 castings from those undesirable strains to which they are subjected by reason of the chilling process. However, so far as I am aware, this property of cast iron to become permanently expanded under certain conditions of heat treatment, has never been utilized in the fitting of a cast iron article to another body with which it is to coöperate.

My invention differs from the ordinary process of annealing metals in a number of 100 respects. The annealing process has for its purpose to change the texture and physical qualities of the metal, and that is all. If it should be proven to be a fact that annealed articles are slightly larger after the annealing process than they were before, and as to this I am not informed, this is and has been a negligible factor, and one hitherto quite or almost entirely overlooked and unknown. On the other hand, in the practice of my invention, the change in the size of the article, due to the heat treatment to which it is subjected, is the object sought, and any change 110 in its physical or molecular condition, due to such treatment, is incidental, and negligible. It is common practice in annealing to subject the articles to a heat treatment for a comparatively long time, and to give them one treatment only; whereas in the practice 115 of my invention I have found that it is not necessary that the heat treatment should be long continued, it being only necessary to uniformly heat the article throughout and bring it up to a red color, immediately after which it is allowed to cool. Moreover, ac- 120

cording to my process, the heat treatment of a particular article may be, and in practice often is, repeated to get successive expansions and added enlargements of the article, 5 the desired increase in size being thus obtained through a stepping-up process. In operating upon comparatively small articles, such as the pistons of gas engines where the volume of metal in each is not large, the 10 length of time required to heat the article to the necessary degree is short; and as herein pointed out, if the temperature be raised only to approximately 1200°, a very slight enlargement takes place. Thus by heat 15 treatment alone an exceedingly accurate fit of a cast iron article to the space it is to occupy, or to another article with which it is to be used, may be quickly and cheaply secured, the successive treatments permitting it to be 20 gradually brought up to the desired size.

This case is a division of my application No. 54,613, filed October 7, 1915.

What I claim is:—

1. The herein described improvement in 25 the art of permanently heat-expanding cast iron which consists in heating the metal to a red heat and then, immediately after the metal has been uniformly heated to the desired degree, uniformly cooling it.
2. The herein described process of causing 30 the permanent expansion of iron castings which consists in bringing them to a red heat, then after the castings have been brought to the desired degree of heat, imme-

dately allowing them to cool, and alternately repeating the said heating and cooling steps to successively expand the articles to the desired degree. 35

3. The herein described improvement in the art of fitting cast iron pistons to cylinders in which they work, which consists in permanently expanding a finished piston to the desired size by subjecting such piston to a heat treatment in which its temperature is raised to the required degree, within the 40 range of temperatures indicated by a red color of the metal, to give the expansion and enlargement desired, and when this temperature has been attained uniformly throughout the piston, then immediately cooling it. 45

4. The herein described improvement in the art of fitting a cast iron piston to a cylinder in which it is to work, which consists in permanently heat-expanding the piston nearly to the desired size by heating it to a 50 red color uniformly throughout and then cooling it, and then subjecting it to a further permanent heat expansion by which it is brought to the desired working size. 55

5. The herein described process of causing 60 the permanent expansion of an iron casting which consists in heating the casting uniformly throughout to a temperature between 1400 and 1600 degrees F. and then immediately after such uniform heating has been 65 attained cooling the article.

WILLIAM A. KNAPP.